

## UNITED STATES PATENT OFFICE

2,108,386

## LUBRICANT PREPARATION

John M. Musselman, Cleveland, and Elliott B. McConnell, Shaker Heights, Ohio, assignors to Standard Oil Company, Cleveland, Ohio, a corporation of Ohio

No Drawing. Application November 14, 1935.  
Serial No. 49,824

7 Claims. (Cl. 87-9)

Lubricating oils where subjected to high temperatures on ferrous base surfaces deteriorate quite rapidly. For efficient results therefore, lubricants obviating this have been much desired.

5 We have now found that compositions of oils and certain glycid oxy-hydrogen compounds present remarkable resistance against such deterioration and afford usage in conditions otherwise not satisfactorily met.

10 To the accomplishment of the foregoing and related ends, the invention, then, comprises the features hereinafter fully described, and particularly pointed out in the claims, the following description and the contained data setting forth in 15 detail certain illustrative embodiments of the invention, these being indicative however, of but a few of the various ways in which the principle of the invention may be employed.

In accordance with the invention, an oil having 20 lubricating viscosity, and a small proportion of a glycid compound are mixed together, the latter compound being of the general formula  $NR_2NCH_2CO.R'(OH)_n$ , in which R is a hydrocarbon radical and R'(OH)<sub>n</sub> a polyhydroxy benzene in which there are at least 2 hydroxyls and in 1,2 position. The oil may be a petroleum oil of viscosity for instance 48 to 200 Saybolt Universal at 25 210° F.

Representative of the glycid compounds are nitrogen-alkyl glycid polyhydroxy benzenes, nitrogen-cycloparaffin glycid polyhydroxybenzenes, nitrogen-alkaryl glycid polyhydroxybenzenes, nitrogen aryl glycid polyhydroxybenzenes, and for instance nitrogen-o-tolyl-glycid-1,2-dihydroxybenzene, nitrogen-m-cyclo-glycid-1,2-dihydroxybenzene, nitrogen-p-isopropyl-phenyl-glycid-1,2-dihydroxybenzene, nitrogen-methyl-glycid-1,2-dihydroxybenzene, nitrogen-cyclohexyl-glycid-1,2-dihydroxybenzene, nitrogen-p-tertiary-butyl-glycid-1,2-dihydroxybenzene, nitrogen-benzyl-glycid-1,2-dihydroxybenzene, nitrogen-alkyl-glycid-1,2-dihydroxybenzene, nitrogen-o-tolyl-glycid-1,2,3-trihydroxybenzene, nitrogen-methyl-glycid-1,2,3-trihydroxybenzene, nitrogen-m-cyclo-glycid-1,2,3-trihydroxybenzene, nitrogen-cyclohexyl-glycid-1,2,3-trihydroxybenzene, nitrogen-p-tertiary-butyl-glycid-1,2,3-trihydroxybenzene, nitrogen-p-isopropyl-phenyl-glycid-1,2,3-trihydroxybenzene, nitrogen-benzyl-glycid-1,2,3-trihydroxybenzene, etc.

50 The glycid derivative, as indicated, is in quite minor proportion. In general it is unnecessary to exceed 1 per cent thereof in the total composition, and proportions as low as 0.01 per cent may be employed, depending somewhat upon the oil and the particular duty in view. The glycid com-

pounds in such amounts dissolve readily in the oil, and by efficient mixing to attain dissemination, the material is correspondingly prepared without recourse to complicated procedure or interference with desirable refinery practice.

5 As an example: With a Mid-Continent neutral lubricating stock having a viscosity of 437 sec. Saybolt Universal at 100° F., there is incorporated 0.01 per cent of nitrogen-para-tolyl-glycid-1,2-dihydroxybenzene.

10 As another example: Similarly with a stock having lubricating viscosity there is incorporated nitrogen-cyclohexyl-glycid-1,2-dihydroxybenzene.

15 As another example: Similarly with a stock having lubricating viscosity there is incorporated nitrogen-benzyl-glycid-1,2-dihydroxybenzene.

20 Other modes of applying the principle of the invention may be employed, change being made as regards the details described, provided the features stated in any of the following claims, or the equivalent of such, be employed.

We therefore particularly point out and distinctly claim as our invention:—

1. A lubricant comprising an oil having lubricating viscosity and a small proportion of a compound of general formula  $NR_2NCH_2CO.R'(OH)_n$ , in which R is a hydrocarbon radical and R'(OH)<sub>n</sub> a polyhydroxy benzene in which there are at least 2 hydroxyls and in 1,2 position.

2. A lubricant comprising an oil having lubricating viscosity and a small proportion of a nitrogen-alkyl-glycid-polyhydroxybenzene in which there are at least 2 hydroxyls and in 1,2 position.

3. A lubricant comprising an oil having lubricating viscosity and a small proportion of a nitrogen-cycloparaffin-glycid-polyhydroxybenzene in which there are at least 2 hydroxyls and in 1,2 position.

4. A lubricant comprising an oil having a lubricating viscosity and a small proportion of a nitrogen-aryl-glycid-polyhydroxybenzene in which there are at least 2 hydroxyls and in 1,2 position.

5. A lubricant comprising an oil having lubricating viscosity and a small proportion of nitrogen-paratolyl-glycid-1,2-dihydroxybenzene.

6. A lubricant comprising an oil having lubricating viscosity and a small proportion of nitrogen-cyclohexyl-glycid-1,2-dihydroxybenzene.

7. A lubricant comprising an oil having lubricating viscosity and a small proportion of nitrogen-benzyl-glycid-1,2-dihydroxybenzene.

JOHN M. MUSSELMAN.  
ELLIOTT B. McCONNELL. 55